

C. DREYmann.

PROCESS OF TINNING METAL PLATES AND OTHER ARTICLES.

APPLICATION FILED MAY 15, 1916.

1,242,532.

Patented Oct. 9, 1917.



*C. Dreymann*  
Inventor

By his Attorneys  
*Ken. Page, Cooper & Hayward*

# UNITED STATES PATENT OFFICE.

CARL DREYmann, OF BALTIMORE, MARYLAND.

## PROCESS OF TINNING METAL PLATES AND OTHER ARTICLES.

1,242,532.

Specification of Letters Patent.

Patented Oct. 9, 1917.

Application filed May 15, 1916. Serial No. 97,507.

*To all whom it may concern:*

Be it known that I, CARL DREYmann, a subject of the German Emperor, residing at Baltimore, in the State of Maryland, have 5 invented certain new and useful Improvements in Processes of Tinning Metal Plates and other Articles, of which the following is a full, clear, and exact description.

In plating sheet iron with tin the bath of 10 molten tin is covered with a layer of palm-oil so that as the tin-coated plate leaves the tin it passes through the oil.

In the process indicated the oil used is 15 consumed in large amount, and I have dis- covered that this is due chiefly to decompo- 20 sition and polymerization of the unsatu- rated fatty acid and glycerid. This decom- position and polymerization increases as the oil is heated, especially when heated to 250° C. or above, the temperature at which the 25 plating with tin is effected. With a glycerid or other ester of a saturated fatty acid, polymerization and decomposition do not occur, or only to a slight extent.

My present invention is based on the 30 above discoveries. In my improved process the "oil" used is a glycerid or ester of a satu- rated fatty acid; as for example oleo-stearin, all kinds of hydrogenated oils and fats, and 35 artificial esters produced from palmitic acid, stearic acid or other saturated acids.

In the accompanying drawing the figure 40 shows diagrammatically a tank or vat A containing molten tin B. The vessel is di- 45 vided by a partition C which terminates above the bottom, thereby dividing the ves- 50 sel into two communicating compartments, D, E. On the molten tin in the latter com-

partment is a body of glycerid or other ester F, and in the former a layer G composed of 40 the usual flux, such as ammonium chloride and zinc chloride.

In carrying out the invention in the pre- 45 ferred manner, the iron plate or sheet pre- 50 viously cleaned in any suitable manner, is passed into the molten tin B in compart- 55 ment D of the vessel A, then under the par- 60 tition C into compartment E, and thence out through the layer of glycerid or other ester F.

The tin plate is equal in every respect to 65 that produced by the palm-oil process, with the important advantage that my process has a much larger output for the same amount of "oil" consumed. In other words, 70 my process is more economical. Experience has shown that the output is at least twenty-five per cent. greater with the same con- 75 sumption of oil.

What I claim is:

1. In a process of tinning metal plates and other articles, the step comprising passing the plate through a bath of molten tin and out through a layer consisting essen- 80 tially of an ester of a saturated fatty acid, 85 floating on the molten tin.

2. In a process of tinning plates and other articles, the steps comprising dipping the plate into a bath of molten tin, and taking the plate out of the bath through a layer or 90 body consisting essentially of hydrogenated oil.

In testimony whereof I hereunto affix my signature.

CARL DREYmann.